

Patented Feb. 10, 1925.

1,525,519

# UNITED STATES PATENT OFFICE.

WILLIAM H. SMITH, OF CLEVELAND, AND CHARLES M. CAMPBELL, OF EAST CLEVELAND, OHIO, ASSIGNEES TO PIONEER ALLOY PRODUCTS COMPANY, OF CLEVELAND, OHIO, A CORPORATION OF DELAWARE.

## MOLD FOR CHROMIUM ALLOYS.

No Drawing.

Application filed September 11, 1922. Serial No. 587,573.

To all whom it may concern:

Be it known that we, WILLIAM H. SMITH and CHARLES M. CAMPBELL, citizens of the United States, residing, respectively, at 5 Cleveland and East Cleveland, in the county of Cuyahoga and State of Ohio, have invented certain new and useful Improvements in Molds for Chromium Alloys, of which the following is a specification.

10 This invention relates to the casting of high chromium alloys and has for its object the provision of a new and improved mold wherein accurate castings can be made without contaminating the alloy. It is known that alloys of chromium with iron group metals are very difficult to cast especially if the proportion of chromium be high and the carbon low. At the elevated temperature required to effect complete 15 fusion of such an alloy, the chromium reacts upon silica, with absorption of silicon and the production of silicon and the production of frothing and blow-holes. The object of our invention is the provision 20 of a mold material which shall produce smooth and regular castings; which shall not materially shrink or expand either upon drying or heating; which shall be made by exactly the same processes as in stand- 25 ard foundry practice, thus avoiding special training of workmen; which shall be capable of being used over and over again like ordinary sand; while further objects and advantages of the invention will be- 30 come apparent as the description proceeds.

In the performance of our invention we 35 employ magnesite as the primary mold material. This material possesses a brittle and somewhat porous nature, and upon crushing ordinarily produces irregular, jagged 40 particles which when packed together as in the making of a mold produce such a dense and interlocked mass as to be substantially non-porous, especially when mixed with the 45 necessary binder to hold the grains in fixed relation with each other. In order to produce a successful mold by the use of this material we find it necessary first to reduce the particles to a rounded granular 50 shape which shall enable them to be packed together in a solid relation without at the same time producing a non-porous mass. At the same time we have found it desirable to produce uniformly graded mixture

containing grains of different sizes which 55 shall produce a solid mass despite the elimination of the jagged interlocking corners.

In the performance of our said invention we crush this magnesite to a fineness dependent upon the size of the molds which 60 are to be made. For molds of approximately a foot square we find it well to crush the material until all of the same will pass a screen of 16 mesh. The crushed material is then tumbled or rumbled together so that the 65 particles may become rounded by mutual attrition and screened to fineness of say 16 mesh, 20 mesh, 32 mesh and finer. These different finenesses are then mixed together in the proportions of say twenty-five per cent 70 of sixteen mesh, twenty-five per cent of twenty mesh, and the balance thirty-two mesh and finer, care being taken not unduly to break the particles. With these we mix a certain proportion of suitable bind- 75 ing material, for example two per cent more or less of clay (either fire clay or common clay) and two per cent more or less of a starchy material such as corn flour. This mixture is then tempered with water to the 80 desired consistency and packed into molds according to the usual foundry practice. These molds are then baked in a suitable oven to drive off excess moisture owing to 85 the very high temperature of the molten metal, thereby producing a mold of the desired mechanical strength and internal smoothness combined with the desired porosity to enable the ready escape of air and mold gases.

After the metal is poured the casting 90 is removed in the usual manner and the mold material is left in a friable lumpy condition. The lumps are broken down to the original grain size by rumbling. It is 95 also ordinarily desirable to screen the material and re-prepare a graded mixture since the handling will have reduced such a proportion of the same to dust that not all can be reused.

The larger the molds the larger can be the sizes of the grains.

Having thus described our invention what we claim is:

1. A mold for chromium alloys wherein 105 the metal contacting surfaces consist substantially of magnesite.
2. A mold for chromium containing al-

- loys made essentially of crushed magnesite and a binder.
3. A mold for chromium containing alloys made essentially of crushed magnesite mixed with a small portion of clay.
4. A mold for chromium-containing alloys made essentially of crushed magnesite, clay, and starchy material.
5. A mold for chromium containing alloys made of a graded mixture of rounded grains of acid-free, basic material having the herein essential properties of magnesite mixed with sufficient binder to hold the grains together without overcoming the porosity of the mass.
6. A composition of matter for making molds for chromium containing alloys, consisting essentially of a graded mixture of rounded grains of magnesite mixed with a small proportion of binding material.
7. Process of producing molds for chromium containing alloys which contains the steps of crushing magnesite to granular form, rumbling the grains to round their corners, adding a suitable binder, and tamping into molds.
8. Process of producing molds for chromium containing alloys which contain the steps of crushing magnesite to granular form, rumbling the grains to round their corners, segregating the different sizes, remixing in suitable proportions to produce a graded mixture, adding a suitable binder, tamping the mixture into molds, and drying.

In testimony whereof, we hereunto affix our signatures.

WILLIAM H. SMITH.  
CHARLES M. CAMPBELL.